

## UNITED STATES PATENT OFFICE

2,457,586

## GREASE COMPOSITION

John F. McGrogan, Philadelphia, Pa., assignor to  
 The Atlantic Refining Company, Philadelphia,  
 Pa., a corporation of Pennsylvania

No Drawing. Application September 4, 1946,  
 Serial No. 694,833

6 Claims. (Cl. 252—36)

1

The present invention relates to improvements in calcium base grease compositions; and particularly those which are utilized in high temperature lubrication or under conditions where the parts lubricated are subject to water washing and/or elevated temperatures. The greases of the present invention are especially applicable in the lubrication of the bearings of rolling mills fabricating hot or cold rolled steel sheets, strips, bars and the like, where the bearings may be water-cooled and therefore subject to the washing action of water. The improved greases are also adapted in the lubrication of wheel bearings, universal joints, and other machine parts where the use of ordinary grease is ineffective due to water solubility or low dropping point.

It is therefore an object of this invention to provide improved calcium base greases characterized by their stability at temperatures well above those at which the ordinary calcium base greases are applicable, and under conditions where the ordinary soda base greases of high dropping point are ineffective due to their water solubility.

Conventional calcium base greases are unsuitable for use at elevated temperatures since they are unstable at temperatures of the order of 200° F. to 220° F., and in many cases lubrication is required at much higher temperatures, for example, at 250° F. to 350° F. in rolling mill bearings.

This invention is predicated upon the fact that by compounding in a calcium base grease, a small amount of a lead salt of an aliphatic monocarboxylic acid of not more than 8 carbon atoms, an improved grease is obtained which possesses not only the desirable characteristics of calcium base greases but also a stability at temperatures much in excess of those at which ordinary calcium base greases are capable of being applied.

In accordance with the present invention, there is incorporated in a calcium base grease comprising lubricating oil and calcium soaps of fatty acids, a small but sufficient amount of a lead salt of the type aforesaid to substantially increase the dropping point of the grease, as determined by the A. S. T. M. method D566-42 entitled "Dropping point of lubricating greases." In general, the improved grease may comprise about 5% to 50% by weight of calcium soaps of fatty acids, 1% to 20% by weight of lead salt, and the balance lubricating oil. Preferably the grease will comprise 10% to 30% of calcium soaps, 1% to 10% of lead salt, and the remainder mineral lubri-

2

cating oil. The calcium soaps may be obtained by saponifying fats such as tallow, fish oil, hog fat, hoss fat (70% oleic acid—30% stearic acid), cottonseed oil, or lard oil with a basic compound of calcium, such as lime flour or hydrated lime, or by neutralizing saturated or unsaturated fatty acids of from 12 to 20 carbon atoms, or mixtures thereof, with lime. The consistency of the improved grease may be varied as desired by increasing or decreasing the calcium soap content, or conversely by varying the amount of lubricating oil used, the consistency being determined by the A. S. T. M. method D217-44T entitled "Consistency of lubricating greases and petrolatum." The dropping point of the grease may be varied, depending upon the quantity of lead salt employed. Conventional calcium base greases usually have dropping points between 180° F. and 230° F., whereas the improved greases of the present invention may have dropping points as high as 500° F. In compounding the grease, it is preferred to employ a lead salt such as lead acetate, although the lead salts of the other aliphatic monocarboxylic acids containing up to 8 carbon atoms will produce similar results, the effect being somewhat less pronounced with increase in carbon atom content.

The present invention may be further illustrated by the following examples, which, however, are not to be construed as limiting the scope thereof.

Greases of various soap content and lead salt content were prepared according to the following procedure, which represents one of several methods which may be employed in compounding the product.

About 10% of the total lubricating oil to be employed is introduced into a steam jacketed grease kettle provided with a mechanical stirrer. The oil is heated, with agitation, and the entire quantity of fat or fatty acid is added and brought into solution in the oil. A slurry of about equal parts of lubricating oil and dry lime is made up, the lime being in the amount necessary to effect saponification of the fat or neutralization of the fatty acids employed. The oil-lime slurry is then added to the oil and fat or fatty acids in the kettle and the temperature of the mixture is maintained between 200° F. and 220° F. until saponification or neutralization is complete, the entire mixture being agitated during this step. The temperature is then increased to about 250° F. to drive off water, if any is produced during the soap-forming step, and about 3/4 of the lubricating oil remaining is added to the oil-soap

mixture in the kettle. The mixture is thoroughly agitated, and the desired amount of lead salt is added, preferably in the form of an aqueous solution of lead acetate having an acetate concentration of about 60% to 70%. The temperature of the mixture is maintained at about 250° F. to drive off all of the water, and the remaining  $\frac{1}{4}$  of the lubricating oil is added and thoroughly incorporated by agitation. The quantity of lubricating oil employed determines the consistency of the product, and as pointed out hereinbefore, may be varied as desired. The hot mixture is cooled to a temperature of the order of 80° F. to 100° F. and the resulting grease is introduced into suitable containers. The ingredients and the properties of the greases are tabulated below.

|                                                                   | 1    | 2    | 3    |
|-------------------------------------------------------------------|------|------|------|
| <i>Ingredients, Wt. Per Cent</i>                                  |      |      |      |
| 300 Paraffin Oil (24° grav., 305" S. U. Vis./100° F., 0° F. pour) | 64.3 | 0    | 0    |
| 100 Paraffin Oil (27° grav., 100" S. U. Vis./100° F., 0° F. pour) | 0    | 31.1 | 23.4 |
| 55 Maltha Oil (19° grav., 155" S. U. Vis./210° F., 30° F. pour)   | 0    | 50.8 | 38.3 |
| Hog fat                                                           | 12.2 | 5.7  | 12.0 |
| Hoss fat                                                          | 11.9 | 5.7  | 12.0 |
| Hydrated lime                                                     | 3.5  | 1.5  | 4.3  |
| Lead acetate $Pb(C_2H_3O_2)_2 \cdot 3H_2O$                        | 8.1  | 5.2  | 10.0 |
| <i>Properties of Product</i>                                      |      |      |      |
| Penetration A. S. T. M. @ 77° F.                                  | 315  | 400+ | 298  |
| Dropping point A. S. T. M., °F.                                   | 473  | 390  | 493  |
| Water Content                                                     | NH   | NH   | NH   |

In the above examples, certain definite proportions of ingredients have been set forth. Such proportions may be varied considerably in order to obtain greases of different consistencies and dropping points. The source of the fats or fatty acids may also vary, as may the technique of compounding the ingredients. The lubricating oils may be of any desired viscosity, for example, from 50" S. U. at 100° F. to 1000" S. U. at 210° F., and may be straight run lubricating distillates or residuums, selective solvent treated oils, cracked oils, hydrogenated oils, oils produced by polymerization of olefins or by alkylation of aromatic hydrocarbons, dewaxed oils, acid treated oils, deasphaltized residual oils, and the like. In general, there may be produced in accordance with this invention, grease compositions having dropping points above about 200° F., and preferably between 300° F. and 500° F., suitable for use at elevated temperatures and/or in the presence of water.

I claim:

1. A grease composition consisting essentially of mineral lubricating oil, calcium soaps of fatty acids in an amount sufficient to impart the desired consistency to the grease, and a small quantity of a lead salt of an aliphatic monocarboxylic acid containing not more than 8 carbon atoms sufficient to increase the dropping point of said grease to a temperature between 300° F. and 500° F.

2. A grease composition consisting essentially of mineral lubricating oil, 5% to 50% by weight of calcium soaps of fatty acids, and from 1% to 20% by weight of a lead salt of an aliphatic monocarboxylic acid containing not more than 8 carbon atoms.

3. A grease composition consisting essentially of mineral lubricating oil, 10% to 30% by weight of calcium soaps of fatty acids, and from 1% to 10% by weight of a lead salt of an aliphatic monocarboxylic acid containing not more than 8 carbon atoms.

4. A grease composition consisting essentially of mineral lubricating oil, calcium soaps of fatty acids in an amount sufficient to impart the desired consistency to the grease, and a small quantity of lead acetate sufficient to increase the dropping point of said grease to a temperature between 300° F. and 500° F.

5. A grease composition consisting essentially of mineral lubricating oil, 10% to 30% by weight of calcium soaps of fatty acids, and 1% to 10% by weight of lead acetate.

6. A grease composition produced by compounding together:

|                         | Per cent |
|-------------------------|----------|
| Mineral lubricating oil | 60-80    |
| Hog fat                 | 5-12     |
| Hoss fat                | 5-12     |
| Lime                    | 1.5-4.5  |
| Lead acetate            | 5-10     |

JOHN F. McGROGAN.

#### REFERENCES CITED

The following references are of record in the file of this patent:

#### UNITED STATES PATENTS

|    | Number    | Name              | Date          |
|----|-----------|-------------------|---------------|
| 50 | 2,197,263 | Carmichael et al. | Apr. 16, 1940 |
|    | 2,399,063 | Schantz           | Apr. 23, 1946 |

#### FOREIGN PATENTS

|    | Number | Country       | Date |
|----|--------|---------------|------|
| 55 | 9,973  | Great Britain | 1900 |